# EUROPEAN PATENT APPLICATION

(11) **EP 0 077 588 A1**
(43) Date of publication of application: **27.04.1983**
(21) Application number: 82201271.2
(22) Date of filing: 12.10.1982
(51) Int. Cl.: C11D 3/37, C11D 3/22, C11D 3/00

(54) **Improved machine dishwashing and rinsing composition**

(30) Priority: 16.10.1981 GB 8131205
(71) Applicant: UNILEVER N.V., 3013 AL Rotterdam (NL); UNILEVER PLC, London EC4P 4BQ (GB)
(72) Inventor: Los, Leendert, NL-3262 NA Oud-Beyerland (NL); Gouda, Johannes Hendrikus, NL-3133 AH Vlaardingen (NL)
(74) Representative: van Gent, Jan Paulus

(57) **Abstract**

Machine dishwashing and rinsing compositions are provided having improved foam control properties by inclusion of an effective amount of a special group of polymers, which consists of polyelectrolytes containing cationic charges and having a cationic charge to carbon atom in the backbone ratio of from 0.03 to 0.5 and a molecular weight in the range of from 5.10³ to 5.10⁵. A typical example of such a polyelectrolyte is the copolymer of N-vinylpyrrolidone and quaternized diethylaminoethylmethacrylate.

## Description

The present invention relates to an improvement in machine dishwashing and rinsing compositions.

In machine diswashing processes usually two products are applied, i.e. a machine dishwashing composition for use in the main wash cycle, and a rinse aid composition for use in the rinse cycle. Both products usually contain an active detergent material. Since both products are applied to the articles to be cleaned or rinsed by spraying the wash or rinse liquor containing these products thereon, which implies the use of a pump, the generation of too much foam thereby is a serious problem. Too much foam can cause too much noise, may damage the heating coil of the dishwashing machine, can lead to the pump malfunctioning and may impair the overall efficacy of the dishwashing process. Consequently, only low-foaming active detergent materials are commonly used in machine dishwashing and rinsing compositions. Nevertheless, still too much foam can be generated, e.g. by the soil removed from the articles to be cleaned, if no additional measures, such as the use of foam depressing agents are taken. This foam formation can cause the pressure of the pump with which the wash liquor or the rinse water is sprayed upon the articles to be cleaned to drop, which produces the above-mentioned disadvantages.

It is therefore an object of the present invention to provide for a machine dishwashing or rinse composition which, when in use in a dishwashing or rinsing operation, prevents the pump pressure from dropping to any significant degree.

It has now been found that this object can be achieved by the inclusion in a machine dishwashing or rinsing composition of a small, effective amount of a special group of polymers. The machine dishwashing or rinsing composition, in which the special group of polymers is included , is of the usual type and formulation, containing as active detergent material a nonionic detergent, preferably a low-foaming one.

In its broadest aspect therefore, the invention relates to a machine dishwashing or rinsing composition comprising a nonionic detergent, and is characterized by the inclusion therein of a small, effective amount of a special group of polymers.

The special group of polymers consists of polyelectrolytes which contain cationic charges, either permanent or at the pH of usage. They have a cationic charge to carbon atom in the backbone ratio of from 0.03 to 0.5. They may contain additional neutral or anionic groups, with an anionic to cationic group ratio of as high as- 3 : 1. They have a molecular weight in the range of 5.10³ to 5.₁₀5_{.}

The special group of polymers consists of three kinds of polymers, i.e. those based on quaternized diethylaminoethylmethacrylate, those based on dimethyldialkylammo- niumhalide, and quaternized polysaccharides.

To the first class belongs as typical example a copolymer of N-vinylpyrrolidone and quaternized diethylaminoethylmethacrylate, having a molecular weight of 10⁵.

To the second class belong as typical examples poly(di- methyldiallyl ammonium chloride) having a molecular weight of 10⁵, and poly(dimethyldiallyl ammonium chloride-acrylamide) having a molecular weight of 2.5 x 10⁵ to 5 x 10⁵ and having a molar percentage ratio of dimethyl- diallyl ammonium chloride to acrylamide ranging from 20 : 80 to 80 : 20. To this second class also belongs 1,5-dimethyl-1,5-diazaundecamethylene-polymetho- bromide, having a molecular weight of 5.10³⁻10⁴.

To the third class belong 2-hydroxypropyl trimethyl ammonium chloride ethers of hydroxyethyl cellulose, having a molecular weight of 10" - 2.₅ x ₁₀⁵.

Typical, commercially available polymers belonging to the above classes are Gafquat 734 ex Gaf Corp.; Merquat 550 ex Chemviron, Brussels, Belgium; Polybrene ex Aldrich Chemical Co., Milwaukee, Wisc., USA; Polymer JR 125 and Polymer JR 400 ex Union Carbide, etc.

The polymers of the invention are used in the machine dishwashing or rinsing composition in an amount of 0.1 to 10%, preferably 0.2 to 1% by weight.

The balance of the composition consists of the usual ingredients, present in machine dishwashing or rinsing compositions.

Thus, the machine dishwashing composition usually comprises from 0.1 to 10 % by weight of a nonionic detergent, preferably a low-foaming one. This is a well-known class of nonionic detergents, examples of which are amply described in the textbook "Nonionic Surfactants" by M. Schick. Furthermore, it comprises from 1 to 80% by weight of one or more builder salts, such as alkali metal-ortho-, -pyro-, -tripoly-, -hexametaphosphates, alkali metal citrates, alkali metal carbonates, alkali metal carboxy methyloxysuccinate, alkali metal nitrilotriacetate, zeolites and so on. In addition, it contains from 1 to 80 % of an alkalimetal silicate, from 1 to 50 % of an oxygen or chlorine bleaching agent, and it may further contain as optional ingredients perfumes, germicides, corrosion inhibitors, enzymes, bleach precursors, reducing agents, clays, and so on. Buffer salts, such as borates, can also be included.

A rinse composition usually also comprises from 1 to 60%, preferably 10 - 35% by weight of a nonionic-detergent, preferably a low-foaming one, and furthermore optional ingredients, such as solvents, (in)organic acids, preservatives, perfumes, dyes, hydrotropes, enzymes, germicides, all in the usual amounts.

It has been found in this respect that it is of specific advantage if the rinsing composition also contains a low level, i.e. 0.1 - 1% by weight of an anionic detergent. The benefits of the present invention are thereby significantly increased in a rinse composition. The anionic detergent can be any well-known type, including fatty acid soaps. Typical examples are alkylaryl sulphonates, alkane sulphonates, olefin sulphonates, alkylsulphates, alkylethersulphates and so on.

Preferred anionic detergents are the alkali metal salts of straight chain C₁₀-C₁₈ akylbenzene sulphonates, and alkali metal salts of C₁₀-C₁₈ alkylether sulphates, containing from 1 - 10 moles of alkylene oxide. Alkylether carboxylates are also suitable.

The compositions of the present invention can be made in any suitable physical form, such as powders, granulates, tablets, liquids, etc. For machine dishwashing products the granular form is usually prepared, whereas the rinse composition is usually in liquid form. In the latter case, the various ingredients of the rinse composition can naturally also be added to the rinse water.

The invention will further be illustrated by way of Example.

### Examples A -F

In the following Examples A - F a normal washing procedure was carried out in a commercial domestic dishwashing machine. In the main wash 30 g of a current commercial dishwashing composition was used and at the start of the final rinse cycle 2 ml. of a liquid rinse aid of the following composition were added:

The tests were carried out with this rinse aid composition as well as with this composition to which either an anionic detergent, a polymer or both were added. The anionic detergent was sodiumdodecylbenzenesulphonate, and the polymer was Gafquat 734, a copolymer of N- vinylpyrrolidone and quaternized diethylaminoethylmethacrylate, having a molecular weight of 10⁵.

The number of rotations per minute of the lower spray-arm of the dishwashing machine was counted at different temperatures. A decrease in the number indicates a drop in pump pressure; if the number of rotations remains constant, the pump pressure remains constant. The following results were obtained:

### Example A

### Example B

### Example C

### Example D

### Example E

### Example F

### Example G

Glass objects were washed in a commercial dishwashing machine using in the main wash 35 g of the following main wash product:

This was repeated, but then with the same composition to which 0.3 % of Gafquat 734 was added. The appearance of the glass objects with regard to the presence of spots thereon after drying was then assessed according to the following score:

After one wash, the following results were obtained:

After four washes:

A rinse cycle with a base product according to Examples A - F, compared with this base product to which 10 % Gafquat 734 was added, gave the following results:
one rinse cycle four rinse cycles

### Example H

A machine dishwashing operation was carried out in a commercial dishwashing machine using the same main wash composition as in Example G at a concentration of 3 g per litre.

Comparison was made in an indentical manner but now using the same main dishwashing composition, to which 0.5% of Gafquat 734 was added.

The number of rotations per minute of the lower spray-arm was counted at different temperatures, and the following results were obtained:

### Rotational speed of spray-arm

## Claims

1. A machine dishwashing or rinsing composition comprising a nonionic detergent, characterized in that it contains 0.1 - 10% by weight of polyelectrolytes containing cationic charges and having a cationic charge to carbon atom in the backbone ratio of from 0.03 to 0.5 and a molecular weight in the range of from 5.10³ to 5.10^{5.}

2. A composition according to claim 1, characterized in that the polyelectrolytes further contain neutral or anionic groups, with an anionic to cationic group ratio not greater than 3 : 1.

3. A composition according to claim 1 or 2, characterized in that it contains from 0.2 to 1% by weight of the polyelectrolytes.

4. A composition according to any of the preceding claims, characterized in that the polyelectrolytes are based on quaternized diethylaminoethylmethacrylate, diethyldialkylammonium halide or quaternized polysaccharide.

5. A machine dishwashing composition according to any of the preceding claims, characterized in that it further comprises:
(i) 0.1 - 10% by weight of a nonionic detergent,
(ii) 1 - 80% by weight of a builder salt,
(iii) 1 - 80% by weight of an alkalimetalsilicate,
(iv) 1 - 50% by weight of a bleaching agent.

6. A rinse composition according to any of the claims 1 - 4, characterized in that it further comprises 1 to 60%, preferably 10 to 35% by weight of a nonionic detergent.

7. A rinse composition according to claim 6, characterized in that it further comprises from 0.1 to 1% by weight of an anionic detergent.

8. A composition according to any of the preceding claims, characterized in that the polyelectrolyte is a copolymer of N-vinylpyrrolidone and quaternized diethylaminoethylmethacrylate.
